

## UNITED STATES PATENT OFFICE

2,093,852

SHEET ABRASIVE MATERIAL AND METHOD  
OF MANUFACTURING THE SAMEFritz Simon, Hamburg, Germany, assignor to  
Norddeutsche Schleifmittel-Industrie, G. m.  
b. H., Altona-Lurup, GermanyNo Drawing. Application December 20, 1934,  
Serial No. 758,440

1 Claim. (Cl. 51—278)

This invention relates to abrasive products, and more particularly, to a new method of manufacturing waterproof abrasive paper.

The general object of the invention is to provide an abrasive surface for use with a backing or supporting material, so that the surface will be capable of improved abrasive action during a longer life than has been the case with abrasive surfaces employed heretofore.

10 A further feature of the invention provides for processing a backing material to make it waterproof and for applying thereon in separate steps, an adhesive base and an abrasive material, the material being bound not only to the base, but to adjacent particles of a bonding material, in order to form a more durable surface.

20 A feature of the invention resides in providing a binder, such as copal and/or resin, in combination with an abrasive, such as grains of silicon carbide, upon a base material mounted upon a backing, whereby the copal and/or resin can be melted to bind together the grains of silicon carbide.

25 In the manufacture of abrasive paper, it is often desirable to provide a product which is waterproof and hence, capable of use on wet surfaces. A further feature of the invention, therefore, provides for treating paper or fabric with sulphuric acid prior to application thereon of base and abrasive layers. Applicant further discovered that in order to render the paper or fabric more pliable, upon the completion of the sulphuric acid bath, a further bath in a solution 30 of grape sugar or starch sugar and glycerin 35 would constitute a distinctive advantage, and this constitutes another feature of the invention.

40 After the paper or cloth has been suitably conditioned, applicant applies an oil base of suitable character which may contain lac, rubber, drying oils and other materials, which, in combined form, comprise a binding agent.

45 In ordinary practice, the abrasive is added, in powdered form, and in sprinkled condition, over the surface of the binder layer. The paper or cloth bearing the binder layer with the abrasive thereon is then baked or otherwise suitably subjected to a temperature over 212 degrees F. This will cause a finished product with a relatively durable surface to result. However, the 50 abrasive particles, when subjected to hard usage, will be rubbed off the surface of the paper or cloth and soon make it unfit for further use. The problem of making the surface more durable 55 by imparting a feature which will enable longer abrasive action to be obtained has been solved

by applicant by simple yet highly novel changes in the binder and abrasive layers.

Thus, applicant's base may consist of glue material, lac, oil, rubber, and other suitable materials well known in the art. However, the use of copal and/or resin or similar materials in the base or binder layer is omitted. The copal is added with the abrasive or grinding material in a mixture spread upon the base. As a result, in practice, there will be a distribution of copal grains between the grains of grinding or abrasive material such as silicon carbide. Since copal will melt at the relatively high temperatures to which the paper is subjected in the baking operation, while the abrasive particles will remain unaffected, it results that upon passing the treated paper or cloth over a hot plate, or otherwise subjecting it to the application of heat, the copal will melt and bind the silicon carbide or other abrasive particles together, so that when the surface is subjected to abrasion, the silicon carbide particles or the like will not rub off as easily as when there is no binder between them. In effect, applicant is adding an element to the abrasive surface 25 which will not affect the abrasive action but will bind the particles of abrasive material together and also tenaciously bind them to the base.

For purposes of improving the binding power of scattered abrasive on a base surface, applicant, in a modified form of the invention, may first apply a very fine powder of resin, copal or the like, to a base surface. A further powder comprising mixed resin or copal and scattered abrasive may be applied thereon and subjected to a heating action. 30 Further application of mixtures of resin or copal in powdered form with abrasive, may be applied and the paper or cloth repeatedly conducted over a hot surface. Finally, the abrasive alone may be applied, since sufficient resin or copal is imbedded in the surface to grasp the abrasive particles firmly, and at the conclusion of the baking or heat application steps, and the consequent hardening of the copal or resin, the abrasive particles will be firmly gripped. By utilizing 35 copal, resin, or the like, in the surface layer, a binder action between the abrasive particles and between the abrasive particles and the oil base 40 surface will be achieved superior to that heretofore obtained.

No disadvantages result from the omission of 50 copal, resin, or the like, from the base layer, and, on the contrary, by using such materials in combination with the abrasive, any desired quantity thereof may be employed necessary for binding 55 together a maximum quantity of abrasive

material; and this amount should be sufficient to obtain the required adhesion between the abrasive particles themselves and between the particles and the base. In practice, the following steps would be employed in carrying out the invention.

1. A suitable paper or cloth would be passed through a bath of concentrated sulphuric acid, then through a bath of water, and then through a solution of grape sugar or starch sugar and glycerin.

2. A layer of oil of desired character, lac, rubber, glue material, etc. For purposes of increasing the elasticity of the adhesive layer, it may be desirable to add castor oil, caoutchouc, etc., in combination with vulcanization accelerators.

3. Sprinkling resin, copal, or the like, in powdered form, plus abrasive, or first resin and the like and then abrasive or a combination of resin or the like plus abrasive.

4. Passing over a hot plate into a baking or drying chamber, and, if desired, repeating operation numbered 3, as hereinbefore described.

A principal feature of the process consists in the use and application of particles of copal and also particles of artificial resin. In practice, the artificial resin comprises the material "bitumina", an asphalt product.

The advantages resulting from applicant's new method of producing abrasive paper are many-fold. The omission of resin or the like from the binder or base layer enables applicant to use an initial layer of great fluidity. The initial layer being less viscous than those formerly employed in which resin constituted an important component enables it to be laid on mechanically; and the spreading is more even and more easily accomplished than with more viscous compositions. Further, with the use of a viscous substance, the paper is easily torn in handling, whereas with applicant's base material of greater fluidity, such tearing is virtually impossible. Yet, the required viscosity necessary for assuring final binding action is obtained when the resin is sprinkled upon the base layer in the subsequent step. This sprinkling of resin upon the base layer, alone or in combination with the abrasive particles, provides a relatively thick durable product obtainable in a single addition of 50 the resin and abrasive particles to the base layer.

In former operations, the thickness of the binder layer depended upon the degree of fluidity of the resin composition contained therein. Thus, if it was desired to obtain a layer of one milli-

meter thickness, for example, it was necessary first to apply a base layer one-half millimeter thick upon which abrasive material was scattered. Then, another binder layer one-half millimeter thick was necessarily applied and abrasive material then scattered upon the subsequent layer. In this way, the required thickness was built up. Such procedure was exceedingly time consuming, because each layer of the resin composition required substantially fifteen hours for 10 drying, before the subsequent layer could be added. In applicant's process, to the contrary, where a relatively non-viscous initial layer is employed, as compared to the resin compositions of high viscosity, the drying takes about four 15 hours instead of fifteen. Furthermore, this initial layer need not be dry in order to receive the powdered resin and abrasive material. Thus, the drying process may take place after the application of both base layer and the powdered 20 material (resin and abrasive material) and the whole is then dried in four hours as compared to fifteen for each layer in the former process. With applicant's improved method, the finished product may be built up to the desired thickness 25 by the proper addition of the powdered resin and particles in one sprinkling operation. No regard to viscosity of initial layers, which determines the thickness of such layers, is necessary, as heretofore pointed out. Moreover, while the former 30 method which required placing one layer on top of another necessarily required that particles of abrasive material be limited to certain size, depending upon the thickness of the base layer, in order to secure a well bonded abrasive surface, in 35 the present instance, such limitation is not present, so long as the abrasive particles and resin particles are arranged to form a surface of desired thickness and evenness subsequent to the baking or drying process, in which the resin melts 40 to hold the abrasive particles together and to the base surface.

I claim:

A method of processing sheet material, consisting in passing the material through a bath of 45 sulphuric acid, then passing the material through a bath of glycerin and grape or starch sugar, then coating the material with a binding agent including drying oils, then applying a binding agent thereon, consisting of resin, copal, or 50 the like, then adding an abrasive material to the surface, and finally, subjecting the surface to high temperature.

FRITZ SIMON.